

## UNITED STATES PATENT OFFICE

2,120,503

## BLASTING EXPLOSIVE

Milo A. Nice, Hazleton, Pa., assignor to Hercules Powder Company, Wilmington, Del., a corporation of Delaware

No Drawing. Application August 13, 1936,  
Serial No. 95,841

3 Claims. (Cl. 52—13)

This invention relates to a new and improved blasting explosive, and more particularly to a non-gelatinous blasting explosive of high density.

Blasting explosives comprise, in general, so-called "straight" dynamites, which contain nitroglycerin in mixed absorbent, "ammonia" dynamites, which contain as explosive nitroglycerin, nitrate of ammonia and a mixed absorbent, gelatin dynamites, which contain a colloided mixture of nitroglycerin and nitrocellulose as explosive, and mixed absorbent, and "ammonia" gelatin dynamites, in which a part of the nitroglycerin of a gelatin dynamite is replaced by nitrate of ammonia.

15 Of the above described dynamites, the gelatin dynamite has the greatest density and the highest water resistance, and "ammonia" dynamites the lowest density and poorest water resistance, with "straight" dynamites intermediate between the two.

In the manufacture of "ammonia" dynamites it has been the tendency, in the past, to incorporate as much nitrate of ammonia as possible, because of its cheapness, combined with its properties as an explosive and nitroglycerin substitute. However, such substitution of nitrate of ammonia for nitroglycerin had the added result of decreasing the density of the dynamite. This decrease in density of the dynamite may be, in some cases, desirable, e. g., where a lessened shattering effect of the dynamite is desired, but also may be, in some cases, undesirable, e. g., in loading holes containing water or mud when the density of the dynamite is so low that it will not sink into the water or mud. In the latter cases great difficulty is experienced in loading the bore-hole.

"Ammonia" dynamites, as heretofore manufactured, are made in strengths ranging from 15% to 60%. While my invention is applicable to all these strengths, it is of the most importance in the 40%, 50%, and 60% strengths, since lower strengths are used in much smaller quantities. Customarily, a 40% "ammonia" dynamite, as made heretofore, contains about 14% nitroglycerin and about 37% nitrate of ammonia, a 50% "ammonia" dynamite about 16% nitroglycerin and about 49% nitrate of ammonia, and a 60% "ammonia" dynamite about 20% nitroglycerin and about 57% nitrate of ammonia, in addition to the mixed absorbent. Such dynamites all have a density corresponding to an average of 110 1 1/4" x 8" cartridges per 50 lbs., i. e., a density such that cartridges of such dynamite will not readily sink in water or mud.

In an attempt to increase the density of such dynamites I increased the content of nitroglycerin and decreased the nitrate of ammonia, as follows:

| Percent dynamite | Percent nitro-glycerin | Percent ammonia nitrate |
|------------------|------------------------|-------------------------|
| 40               | 22                     | 26                      |
| 50               | 24                     | 37                      |
| 60               | 28                     | 46                      |

and found that I thereby obtained a density corresponding to 106 1 1/4" x 8" cartridges per 50 lbs., or a density of such that such cartridges will not readily sink in water or mud.

I have found that ammonia dynamites having a density corresponding to about 106 or more 1 1/4" x 8" cartridges per 50 lbs. will not sink readily in water or mud in a borehole, whereas ammonia dynamites having a density corresponding to about 90—100 1 1/4" x 8" cartridges per 50 lbs. will sink readily in water or mud in a bore-hole.

Now in accordance with this invention I have found that by incorporating as little as about 0.1% to about 0.4% of nitrocellulose in the above compositions, I obtain a surprising increase in density, or a number of 1 1/4" x 8" cartridges per 50 lbs. of 90—100, i. e., a density such that cartridges thereof will sink in water or mud. Such densities as the latter render loading of boreholes containing water or mud easy, because this density of such cartridges is such that they sink in water or mud.

This result, i. e., the great increase in density of the "ammonia" dynamites, is quite unexpected and one which I have been unable to explain. The addition of such relatively small quantities of nitrocellulose to the nitroglycerin could affect the specific gravity of the nitroglycerine only inappreciably, yet the dynamites produced therewith exhibit utterly unexpected increases in density. In addition to the advantageous increase in density, I obtain an increased water-resistance of the dynamite, which allows the cartridges to remain under water, without substantial deteriorations, for a much greater length of time than is the case with ordinary "ammonia" dynamites.

It will be appreciated that my improved "ammonia" dynamites of high density are not gelatin dynamites, since they do not have the gelatinous consistency of the latter, and are packed into car-

tridges by the use of a machine used for loading non-gelatinous dynamite, instead of by the use of a squeezer or gelatin packing machine.

As specific examples of my improved, non-gelatinous dynamites containing nitrate of ammonia and of high density such as to sink in water or mud, I give below the following illustrative compositions:

| 10                       | Percent<br>40 | Percent<br>50 | Percent<br>60 |
|--------------------------|---------------|---------------|---------------|
|                          |               |               |               |
| Nitroglycerin.....       | 22.0          | 24.0          | 27.0          |
| Nitrocotton.....         | .2            | .2            | .2            |
| 15 Ammonium nitrate..... | 25.0          | 36.0          | 45.5          |
| Sodium nitrate.....      | 36.7          | 26.3          | 16.4          |
| Wood pulp.....           |               |               | 2.0           |
| Flour starch, etc.....   | 11.6          | 10.0          | 5.4           |
| Sulfur.....              | 4.0           | 3.0           | 3.0           |
| Chalk.....               | .5            | .5            | .5            |

20 Ammonia dynamites in accordance with the above formulae are characterized by a surprising increase in density, e. g. 92-95 1 1/4" x 8" cartridges per 50 lbs., i. e. of such density that cartridges thereof will readily sink in water or mud in a borehole.

It will be appreciated that the above compositions are for illustrative purposes only, and that I may make various modifications thereof without departing from the essence of my invention, which comprises broadly a non-gelatinous blasting explosive of high density comprising a liquid explosive, nitrocellulose, nitrate of ammonia and active mixed absorbent, having a density,

when packed in cartridges, such that said cartridges will sink in water or mud.

What I claim and desire to protect by Letters Patent is:

1. A non-gelatinous blasting explosive comprising an explosive liquid nitric ester, nitrocellulose, ammonia nitrate, and a non-detonating absorbent, and having a density corresponding to from about 90 to about 100 1 1/4" x 8" cartridges per 50 pounds, the ammonium nitrate being present in 10 an amount between about 26% to about 46% of the mixture, and the explosive liquid nitric ester being present in amount between about 22% and about 28% of the mixture.

2. A non-gelatinous blasting explosive comprising nitroglycerin, nitrocellulose, ammonium nitrate, and a non-detonating absorbent, and having a density corresponding to from about 90 to about 100 1 1/4" x 8" cartridges per 50 pounds, the ammonium nitrate being present in an amount 20 between about 26% to about 46% of the mixture, and the nitroglycerin being present in amount between about 22% and about 28% of the mixture.

3. A non-gelatinous blasting explosive comprising nitroglycerin from about 22% to about 27%, 25 nitrocellulose about 0.2%, ammonium nitrate from about 25% to about 45.5%, sodium nitrate from about 36.7% to about 16.4%, wood pulp from 0% to about 2%, flour from about 11.6% to about 5.4%, sulfur from about 4% to about 3%, chalk about 30 0.5%, and having a density corresponding to from about 90 to about 100 1 1/4" x 8" cartridges per 50 pounds.

MILO A. NICE.